

# UNITED STATES PATENT OFFICE.

RADCLYFFE FURNESS, OF JENKINTOWN, PENNSYLVANIA.

## HIGH-SPEED TOOL-STEEL.

1,095,842.

Specification of Letters Patent.

Patented May 5, 1914.

No Drawing.

Application filed January 30, 1914. Serial No. 815,402.

*To all whom it may concern:*

Be it known that I, RADCLYFFE FURNESS, a citizen of the United States, residing at Jenkintown, county of Montgomery and 5 State of Pennsylvania, have invented a new and useful Improvement in High-Speed Tool-Steel, of which the following is a full, clear, and exact description.

The object of my invention is to produce 10 a new and improved high speed tool steel which will endure for a greater length of time at the same cut feed and speed, or which can operate at a higher cut feed and speed and therefore remove more metal in a given 15 length of time, than any high speed tool steel heretofore known.

The invention consists of steel containing vanadium, chromium, tungsten and cobalt in certain definite proportions. The following 20 is a typical composition and one which careful experiment has shown to produce the best results: iron, 74 per cent.; vanadium, 1.5 per cent.; chromium, 3 per cent.; tungsten, 17.5 per cent.; cobalt, 4 per cent. The iron 25 should contain about .65 per cent. of carbon, the proportion of which must not exceed one per cent., and may contain the usual small percentages of natural alloys or impurities, such as manganese, silicon, titanium, phosphorus and sulfur, present in comparatively 30 low carbon steel, the percentage of vanadium should not exceed two per cent. nor be less than one per cent. The cobalt may vary within a range of from three to seven per 35 cent., the chromium within a range of from two and one half to four per cent., and the tungsten within a range of from sixteen and one half to twenty per cent. If the steel contains a proportion of any of the enumerated 40 alloying metals less than the minimum specified, the durability of the steel becomes so pronouncedly affected as to render the same measurably inferior to high speed tool steels of other known combinations of elements. If, on the other hand, the maximum 45 proportions specified are exceeded in any given instance, the same result, together with brittleness, develops. It should also be mentioned that if the proportions of any one of the alloying ingredients specified are increased or diminished beyond or below those 50 of the typical composition above defined, the proportions of the other alloying ingredients should be increased or diminished 55 accordingly, so as to maintain approxi-

mately, although not necessarily exactly, the relative proportions specified. For example, good results would not be obtained by using the maximum percentage of one or more ingredients and the minimum percentage of one or more other ingredients. 60

I am aware that various patents for high speed and other steels have issued, and some literature has been published, in which the use of one or more of all the above ingredients, and even the precise combination of ingredients hereinbefore specified, have been suggested; but such patents disclose no really useful information to those skilled in the art, as the possible relative and absolute 65 percentages of the ingredients are almost infinite, whereas unless the relative and absolute percentages are fixed and determined within narrow limits, no efficient cutting steel would be produced and many steels 70 containing the precise ingredients hereinbefore mentioned as essential to a composition embodying my invention would be worse than worthless for tool steel or for any other purpose. In my invention, on 75 the contrary, any one skilled in the art can produce an effective and superior high speed tool steel without the necessity of any experimentation whatever, the ingredients being mixed and the steel manufactured in no 80 way different from that characterizing other known compositions of high speed tool steel and well known to those skilled in the art. 85

While I have mentioned that the steel above described is adapted especially for 90 high speed tool steel, it is also capable of other uses, as for example any device for working hot metal, such as gripper dies, nut piercers and header dies. For such purposes the steel should contain from .20 to 95 .60 per cent. of carbon.

Having now fully described my invention, what I claim and desire to protect by Letters Patent is:

1. A high speed tool steel containing vanadium, from one to two per cent.; cobalt, from 3 to 7 per cent.; chromium, from 2.5 to 4 per cent.; and tungsten, from 16.5 to 20 per cent. 100
2. A high speed tool steel containing vanadium, about 1.5 per cent.; cobalt about 4 per cent.; chromium, about 3 per cent.; and tungsten, about 17.5 per cent. 105
3. A high speed tool steel containing vanadium, from one to two per cent.; co- 110

balt, from 3 to 7 per cent.; chromium, from 2.5 to 4 per cent.; and tungsten from 16.5 to 20 per cent.; the relative percentages of the vanadium, cobalt, chromium and tungsten 5 being approximately in the ratio of 1.5, 4, 3 and 17.5.

In testimony of which invention I have

hereunto set my hand, at Philadelphia, on this 29th day of January, 1914.

RADCLYFFE FURNESS.

Witnesses:

M. M. HAMILTON,  
E. E. WALL.